

## UNITED STATES PATENT OFFICE.

PAUL CAMPION, OF FOREST-NEAR-BRUSSELS, BELGIUM, ASSIGNOR TO A. B. DICK COMPANY, OF CHICAGO, ILLINOIS, A CORPORATION OF ILLINOIS.

## MANUFACTURE OF STENCILS FOR DUPLICATING APPARATUS.

No Drawing. Application filed December 12, 1921, Serial No. 521,866, and in Belgium December 22, 1920.

This invention relates to the manufacture of stencils for duplicating apparatus, and it has more particularly for its object to provide an improved process for the manufacture of such stencils which will afford considerable advantages compared with the processes employed hitherto, as will be perceived from the following description.

Stencils as employed hitherto have, as a matter of fact, the following drawbacks:—

1. A paraffin-coated stencil allows the duplicating ink to pass through the cracks that are caused accidentally either through the usual handling, or by the stencil being carried along by the type-writing machine in which it is being used, at the instant when it is being impressed by the matter that is to be duplicated. Such cracks give rise to ink spots on the copies.

2. Other kinds of stencils are not subject to the occurrence of the cracks referred to under 1, but they have to be moistened before being used in the typewriter. This moistening operation has as its chief drawback, that of causing the parts of the typewriter to become moistened as well, with consequent rusting and deterioration of those parts. A stencil of that kind is not sufficiently thick (that is, has not sufficient

“body”) and is difficult to keep in correct position on the inking cylinders of rotary and other duplicating machines so that the matter on the stencil is not adapted to produce uniform copies.

The above-mentioned drawbacks are obviated by the present invention which consists broadly in using as the stencil a sheet of Japanese paper (such as is already in general use in this class of manufacture and commonly known as Yoshino) impregnated uniformly with pharmaceutical or industrial collodion, or a solution of celluloid with an addition of castor oil, and coated on one side with a coat of paraffin, ceresine wax, or generally with a coat of a solidifiable fatty mineral, vegetable or animal substance.

This last coat is intended to maintain in a supple condition the collodion or solution of celluloid with which the sheet is impregnated; it also serves as a cushion or resilient underlay for facilitating the stencilizing of

the coat of collodion or solution of celluloid by the type characters of the typewriter.

It is to be noted that with this object in view the typing should be done on that side of the sheet that is not coated with paraffin.

As a bath having a celluloid basis there may be used a suitable solution of this latter substance in one of its solvents, or in several of these together, such as ether, acetone, acetic ether, etc., to which solution there is added a certain amount of castor oil or other suitable similar oil, such that the impregnated sheet shall have the requisite suppleness and thickness. Good results can be obtained by adding approximately 40% of castor oil to a 2½% solution of either collodion or celluloid.

A stencil sheet produced according to this invention possesses “body” and need not be moistened before being typed upon, and it can crack, and even be creased or rumpled without any ink spots getting upon the copies.

The same advantages can obviously be obtained, although in a lesser degree by using two sheets one placed upon the other, the first sheet being simply impregnated with collodion or a solution of celluloid, whereas the other sheet is simply coated with paraffin.

Or a single sheet may be used simply impregnated with collodion or a solution of celluloid, and the supporting foundation or underlay being coated with a coat of paraffin.

## Claims:

1. A type-impressible stencil-sheet having a base such as Japanese Yoshino coated with a homogeneous substance including collodion and a suitable oil.

2. A type-impressible stencil-sheet having a base such as Japanese Yoshino coated with a homogeneous substance including collodion and castor oil.

3. A type-impressible stencil-sheet having a base such as Japanese Yoshino coated with a substance including collodion and castor oil, and, in addition, with a solidifiable material.

4. A type-impressible stencil-sheet having a base such as Japanese Yoshino coated with a substance including a cellulose compound.

and castor oil, and, in addition, with a solidifiable material applied on one side thereof.

5. A type-impressible stencil-sheet having a base such as Japanese Yoshino coated with a substance including a cellulose compound and castor oil, and, in addition, with a waxy material.

6. A type-impressible stencil-sheet having a base such as Japanese Yoshino coated with a substance including a cellulose compound and castor oil, and, in addition, with a waxy material applied on one side of said sheet.

In witness whereof I affix my signature.

PAUL CAMPION.